

Oct. 25, 1932.

J. H. TAYLOR

1,884,914

METHOD OF MAKING NOZZLES

Filed Oct. 4, 1928

2 Sheets-Sheet 1



Inventor  
James Hall Taylor  
By Brown, Jackson, Bottcher &  
Dinner

Atty.s.

Oct. 25, 1932.

J. H. TAYLOR

1,884,914

METHOD OF MAKING NOZZLES

Filed Oct. 4, 1928

2 Sheets-Sheet 2



Inventor

James Hall Taylor

By Brown, Jackson, Borttcher and  
Dinner Attys.

## UNITED STATES PATENT OFFICE

JAMES HALL TAYLOR, OF OAK PARK, ILLINOIS

## METHOD OF MAKING NOZZLES

Application filed October 4, 1928. Serial No. 310,414.

My invention relates to a new and improved method of making nozzles of the type commonly used in connection with steam boilers and consisting of a neck with a flange at each end thereof. More specifically, my invention has to do with what is known as the "high" type of nozzle.

The accompanying drawings illustrate an apparatus suitable for practicing my invention and, step by step, my method from billet to finished article.

In these drawings;

Figure 1 shows the original billet;

Figure 2 shows the result of the first operation on the billet;

Figure 3 is an axial cross-sectional view of the apparatus, showing the billet, in the form of Figure 2, placed therein;

Figure 4 is a partial horizontal sectional view of the apparatus taken on the plane of the line 4-4 of Figure 3;

Figure 5 illustrates, in axial cross section, and on somewhat larger scale, the next operation on the billet; and

Figures 6, 7, 8 and 9 illustrate, in axial cross-section, and on still larger scale, and consecutively, the further operations on the billet, the finished article being shown in Figure 9.

The original billet of wrought iron or steel is shown at 10 in Figure 1. The first operation reduces the central portion of the billet and brings it to cylindrical form, as indicated at 11 in Figure 2, this operation leaving the head 12 at the top, and the head 13 at the bottom, thereof.

The billet, in this form is then placed in a machine which I shall now describe.

The main frame of the machine is of general circular form and is shown at 14. It is provided with a top plate 15 and the central portion of the assembly is in the form of a die-receiving tube 16. The frame is adjustably mounted on standards 17 which, in turn, are supported from pistons 18 operating in cylinders 19 in the base 20. Thus the frame may be raised by pressure in the cylinders and lowered by gravity, as desired.

In the frame 14, four radially disposed die members 22 are mounted, ninety degrees

apart, for inward and outward sliding movement, the inner ends of these members extending into the central tube 16 as shown. The die members 22 are moved by means of vertically movable wedge blocks 23, 23 which operate between them and the rim of the frame 14 and with both of which they engage by means of the tongue and groove interlocks 24 and 24', respectively. On the under side of the frame 14 a plurality of brackets 25 are provided, one for each die member 22, each of them bearing a screw gear 26, and a screw 27, fixedly secured to the respective wedge block 23, engages within this screw gear. A pinion 28 mounted on a shaft 29, also journaled in each bracket 25, meshes with each of the respective gears 26. A pinion 30 carried on the upper end of shaft 29 meshes with the ring gear 31. This ring gear is supported by the annular bracket 32 which also provides a bearing for the upper end of the shaft 29. A worm wheel 33 is mounted on one of the shafts 29 and power is applied thereto through the worm 34 on the shaft of a motor 35 mounted on the under side of the frame. Thus, the four die members 22 may be moved simultaneously inwardly and outwardly by means of the motor 35.

A circular die 37 is disposed in the central tube 16, over the die members 22, and a circular die 38, larger in internal diameter, is inserted therein below them. The stationary platen is shown below the tube at 39 and the movable platen over it at 40.

The billet, in the form shown in Figure 2, is disposed in the machine, within the tube 16, as shown in Figure 3, and the die members 22 are moved inwardly to the position illustrated, i. e., holding the billet at its central portion with which the ends of the die members are substantially commensurate. The heads 12 and 13 then provide the material from which the upper and lower flanges, respectively, are to be made. An upper die 41 carried by platen 40, fits into the circular die 37 and a lower die 42, resting on platen 39, fits into the circular die 38. The circular dies determine the diameter of the flanges of the finished article and they are slightly flared.

as indicated at 37' and 38' for a purpose to be described presently.

The movable platen 40 is brought down to bring the die 41 into the die 37, with die 42 engaging the bottom of the billet. Continued downward movement results in smashing down the two heads into the form shown in Figure 5, thus forming the upper and lower flanges 12' and 13'. It is obvious that in this 10 operation the entire frame 14 must move downwardly somewhat as the lower head of the billet is reduced, this being permitted by the mounting of the frame as previously described.

15 It is also clear that in this operation the die members 22 form a closed die around the central cylindrical portion of the billet and that it is against them that the dies 41 and 42 operate.

20 After the operation illustrated in Figure 5 has been completed, the die members 22 are slightly withdrawn, as shown in Figure 6, to leave a space 44 around the central portion of the billet. The billet is now to be axially 25 pierced, as will be described, and the horizontal area of the annular space 44 is approximately equal to the horizontal area of the piercing. The lower die block 42 is left in place, in this piercing operation, but the upper die block 41 is removed and a guide block 20 45 is inserted in the circular die 37. This guide block guides the piercing tool 46 which is substituted for the die block 41 on the upper platen 40. The piercing tool, which is of a diameter equal to the desired internal diameter of the finished article, is then brought 25 30 downwardly, piercing an axial hole in and almost through the billet, as shown in Figure 7. This results in the outward spreading 35 of the material in the central portion of the billet, filling the space 44, no material being 40 removed in this operation.

25 The piercing tool is then withdrawn, and the guide block 45 is removed if desired, and a punch 50 inserted ahead of the tool in the hole in the billet, as shown in Figure 8.

30 The piercing tool is then again brought down to force the punch through the billet. In this punching operation, however, an annular block 51 is inserted between the billet and the lower platen 42 so that the material removed may be received by it. This forms the tubular neck 11' and completes the nozzle to the form shown in Figure 9. The upper platen is then raised, and the tool and punch are removed and the frame is then raised away from the platen 42. Then the die members 22 are withdrawn and the finished article dropped out of the circular dies, the flaring of the flanges, hereinbefore referred to, and the fact that the lower flange is the larger, permitting the ready release thereof.

I claim:

35 1. The method of making nozzles, which

comprises forming a billet with a reduced mid-portion and end flanges, piercing the billet and thereby displacing and redistributing the metal of the mid-portion radially thereof, and confining the radial extension of said mid-portion to a diameter less than that of either of the flanges, thereby forming an intervening tubular neck between the flanges and of less exterior diameter than either flange.

2. The method of making nozzles, which comprises forming a billet with a reduced mid-portion and end flanges, piercing the billet from one end thereof to within a short distance of its other end and thereby displacing and redistributing the metal of the mid-portion radially thereof, confining the radial extension of said mid-portion to a diameter less than that of either of the flanges, and punching out the metal at said other end of the billet to complete the opening therethrough.

In witness whereof, I hereunto subscribe my name this 28th day of September, 1928.

JAMES HALL TAYLOR.

90

95

100

105

110

115

120

125

130